

Feb. 13, 1940.

R. WARNECKE ET AL  
SECONDARY ELECTRON EMMITTER

2,189,972

Filed April 19, 1939



INVENTOR.  
ROBERT WARNECKE AND ANDRE BRIOT  
BY  
Charles M. McClain  
ATTORNEY.

## UNITED STATES PATENT OFFICE

2,189,972

## SECONDARY ELECTRON EMITTER

Robert Warnecke and André Briot, Paris, France,  
assignors to Compagnie Générale de Télé-  
graphie Sans Fil, a corporation of France

Application April 19, 1939, Serial No. 268,734  
In France April 22, 1938

4 Claims. (Cl. 250—174)

The present invention relates to materials having a high secondary to primary electron emission ratio and primarily useful for electrodes for electron multipliers and similar discharge devices 5 which utilize secondary electron emission.

It is known to coat secondary electron emitters with layers having either an alkaline earth oxide base or with complex layers having a caesium base. The emitters with the oxide base 10 are stable and can be easily prepared, but have a rather low coefficient of secondary electron emission, which is the quotient or ratio obtained by dividing the number of secondary electrons by the number of primary electrons. The emitters having the caesium base have a substantially higher secondary electron emission coefficient, but are difficult to prepare and are susceptible to deterioration on rather slight increases in temperature; furthermore, it is difficult to obtain several identical surfaces which 15 have the same coefficient of secondary electron emission.

The principal object of our invention is to provide a secondary electron emitter which has a greater coefficient of secondary electron emission and substantially as good stability as prior 20 emitters with alkaline earth oxide bases. Another object is to facilitate the making of such emitters.

30 In accordance with our invention we make the surfaces or electrodes of high secondary electron emissivity of a base consisting of alloys of light metals, such as aluminum and beryllium, with the addition of a small amount of ferrous metal, such as iron, and of a metalloid, preferably silicon.

We have found that by adding a small amount of iron and silicon we can obtain alloys which consist predominantly of aluminum and contain up to 30% of beryllium. No prior alloys of this 40 kind which contain more than a small percentage of beryllium are known to us. The addition of the iron and silicon to the alloys of aluminum with beryllium produces a new material, as it seems to modify the physical structure so that 45 it differs from that of the binary alloys, and to impart to the surface a higher power of secondary electron emission than is obtainable from the binary beryllium alloys alone.

The composition of the alloys of our invention 50 may vary within rather wide limits especially in the proportions of beryllium to the other light metal, such as aluminum. For example, the beryllium may constitute from 10% to 30% of the alloy, the iron and silicon addition about 1% to 10%, with the remainder the other light metal,

such as aluminum. The ratio of iron to silicon in the addition may vary widely, although in general it is desirable that the silicon constitute at least half or more of the addition. One specific alloy which we have found to be especially 5 suitable for secondary electron emitters is of the following composition: aluminum 74%, beryllium 21%, iron 2%, silicon 3%.

The accompanying figure shows, as a function of the velocity of the primary electrons expressed in volts, the secondary electron emission coefficient obtained with the above alloy. For a velocity of 400 volts of the primary electrons, the secondary emission coefficient exceeds the value of 5, which is somewhat below the values 10 obtained with complex or caesiated surfaces having a caesium base. On the other hand, emitters made of this alloy in accordance with our invention have marked advantages over the caesiated 15 type because of facility in preparing the electrodes, regularity of the results obtained, and the very high stability; and our emitters also have advantages, as the secondary electron emission obtained from emitters of this alloy is substantially greater than can be obtained from the 20 surfaces with alkaline earth oxide base ordinarily employed.

The preparation of electrodes made from the 25 alloy in accordance with our invention is simple. For instance, the electrode made from such 30 alloy is placed in a glass vessel in which is created a high vacuum (of the order of  $10^{-7}$  millimeter mercury), while the electrode is freed from occluded gases by heating it with high frequency inductive heating or electronic bombardment. 35 No treatment other than degassing in high vacuum is necessary to develop the high secondary electron emissivity.

The electrodes or emitters thus obtained have the advantage of a high thermic stability. They 40 are of particular use in tubes with multiplying emitters or electrodes which dissipate through radiation a rather large amount of energy and which therefore should be able to stand relatively high temperatures such as (300° C.) without 45 losing their emitting properties.

We claim:

1. A secondary electron emitting electrode for 50 electron multipliers and the like having a surface of high secondary electron emissivity and composed of an alloy consisting of 10% to 30% beryllium, 1% to 10% of iron and silicon, and the balance aluminum.

2. A secondary electron emitting electrode composed of an alloy consisting of 15% to 25% beryllium 55

lum, 1% to 10% of an addition consisting of iron and silicon in which the silicon equals or exceeds the iron, and the balance aluminum.

3. A secondary electron emitting electrode composed of 74% aluminum, 21% beryllium, 2% iron and 3% silicon.

4. A secondary electron emitting electrode composed of an alloy consisting of a base constitut-

ing at least 90% of the alloy and composed of aluminum and beryllium and containing at least twice as much aluminum as beryllium, and added metals consisting of silicon and iron, the silicon constituting at least half of the added metals.

5

ROBERT WARNECKE.  
ANDRÉ BRIOT.